

1

3,824,119

PRESSURE SENSITIVE COPY PAPER EMPLOYING  
DIBENZYLAMINO FLUORAN COMPOUNDS

Mutsuo Terayama and Kenji Yamamoto, Yao, Japan, assignors to Yamamoto Kagaku Gosei K.K.  
No Drawing. Original application Mar. 10, 1971, Ser. No. 123,069. Divided and this application Sept. 14, 1972, Ser. No. 288,993

Claims priority, application Japan, July 8, 1970,

45/59,711

Int. Cl. B41c 1/06; B41m 5/00

U.S. Cl. 117—36.2

15 Claims

ABSTRACT OF THE DISCLOSURE

New fluoran compounds containing a dibenzylamino group or a nuclear substituted derivative thereof are provided by a novel method involving the reaction of an aminofluoran and a benzyl chloride in the presence of alkali in an inert non-polar organic solvent. The dibenzylamino fluorans are incorporated as a remarkably effective color former in pressure sensitive copying paper.

This is a division of application Ser. No. 123,069, filed Mar. 10, 1971.

BACKGROUND OF THE INVENTION

Fundamentally, pressure sensitive copying paper consists of two sheets of paper, the lower surface of the upper leaf having applied thereto minute capsules containing a color reactive achromatic substance (hereinafter called "a color former") dissolved in a low volatile solvent and the upper surface of the lower leaf being coated with a solid acid, such as acid clay, phenolic compounds, etc. When the lower surface of the upper leaf and the upper surface of the lower leaf are put together and pressure is applied to the upper surface of the upper leaf by handwriting or typing, the capsules under pressure are broken and the color former contained therein is absorbed by the solid acid on the upper surface of the lower leaf to develop a color, thus providing a copy. There is also a type of pressure sensitive copying paper having a mechanism to develop color when a regional pressure is exerted upon a sheet of paper holding capsules, which contain a color former, and a solid acid on or within it. However, such type is quite similar to the first mentioned pressure sensitive copying paper consisting of two sheets of paper, an upper and lower leaf with respect to the mechanism of color formation, and thus the same color former can be used for both types.

As the color former, various kinds of chemical compounds have been used, and, among others, the fluoran compounds have recently been occupying an important position in the pressure sensitive copying paper industry because of the rich variety of colors that such compounds develop and the high color-developing speeds.

For example, 3,6-dimethoxy fluoran (Beilstein Hauptwerk, Vol. XIX, p. 225) readily develops into yellow; 7-chloro-6-methyl-3-diethylamino fluoran (Japanese Pat. Publn. No. 21,199/1968) into yellowish red; rhodamine lactone (Beilstein Hauptwerk, Vol. XIX, p. 344) into bluish red; and 3-diethylamino-7-methylamino fluoran (Canadian Pat. No. 814,948) into green-brackish green. Among the above-mentioned derivatives and homologues, many of them have become commercially available as dyes for pressure sensitive copying paper.

SUMMARY OF THE INVENTION

We have discovered new fluoran compounds containing a dibenzylamino group or its nuclear substituted derivatives represented by the following general formula I

2

(this compound will, hereinafter, be referred to as dibenzylamino fluoran compound)



(I)

- 15 In the above formula  $R_1$  and  $R_2$  are individually hydrogen, halogen or methyl;  $R_3$  is hydrogen, halogen or lower alkyl;  $R_4$  and  $R_5$  are individually methyl or ethyl; and  $n$  is an integer from 1 to 5.  $R_1$ ,  $R_2$ ,  $R_3$ ,  $R_4$ , and  $R_5$  can be concurrently in any combination. In the case where  $R_1$ ,  $R_2$  or  $R_3$  are halogen, chlorine and bromine are preferred. As a color former for pressure sensitive copying paper, the new fluoran compounds are outstanding in the significant requirements of color developing speed, developed color density, light resistance after color development and solubility thereof. In making the novel pressure sensitive copying paper, the compounds are dissolved in a low volatile solvent and packed in minute capsules which are used in conjunction with a solid acid.

DETAILED DESCRIPTION

30 Unfortunately, known manufacturing methods, when applied to the dialkylamino-dibenzylamino fluorans, are high in cost due to the low yield of end product and the intricacy of the process involved. For purposes of the invention, we have considered it important to eliminate this deficiency. For example, 3-diethylamino-7-dibenzylamino fluoran, among the compounds represented by the general formula (I), may be prepared by a conventional known method as follows:



65 In the equation  $R$  represents hydrogen, methyl or ethyl,  $R_1$ ,  $R_2$ ,  $R_3$  and  $n$  are the same as defined in the general formula I. In this case the compound (A) must first be synthesized, i.e., by dibenzylation of the corresponding amino compound.

70 For the dibenzylation the following methods are known: (1) a reaction with benzyl chloride in alcohol (Beilstein Hauptwerk, Vol. XIII, p. 450); (2) a reaction



White crystals

Yield: 11.0 g. (82% of theoretical value)

Melting point: 109-110° C.

Results of analysis:  $C_{38}H_{32}N_2O_3Cl_2$

Calculated: C, 71.81%; H, 5.04%; N, 4.41%

Found: C, 74.08%; H, 5.08%; N, 4.53%.

#### EXAMPLE 4

Preparation of 3-diethylamino-5-methyl-7-dibenzylamino fluoran (in I,  $R_1=CH_3$ ,  $R_2=R_3=H$ )

13 g. of 3-diethylamino-5-methyl-7-aminofluoran (in II,  $R_1=CH_3$ ,  $R_2=H$ ), 16.5 g. of benzyl chloride, 10 g. of anhydrous potassium carbonate and 100 ml. of toluene are subjected to reaction in a manner similar to that of Example 1.

White crystals

Yield: 9.1 g. (48.3% of theoretical value)

Melting point: 173-174° C.

Results of analysis:  $C_{39}H_{36}N_2O_3$

Calculated: C, 80.69%; H, 6.21%; N, 4.83%

Found: C, 80.01%; H, 6.02%; N, 4.75%.

#### EXAMPLE 5

Preparation of 3-diethylamino-7-di(3'-methylbenzyl) aminofluoran (in I,  $R_1=R_2=H$ ,  $R_3=3'-CH_3$ )

7.72 g. of 3-diethylamino-7-aminofluoran, 11.24 g. of 3-methylbenzyl chloride, 8.2 g. of anhydrous potassium carbonate and 100 ml. of toluene are subjected to reaction in a manner similar to that of Example 1.

White crystals

Yield: 6.5 g. (56% of theoretical value)

Melting point: 174-177° C.

Results of analysis:  $C_{40}H_{38}N_2O_3$

Calculated: C, 80.81%; H, 6.40%; N, 4.71%

Found: C, 80.33%; H, 6.39%; N, 4.57%.

#### EXAMPLE 6

Preparation of 3-diethylamino-7-bis(2' 4'-dimethylbenzyl)aminofluoran (in I,  $R_1=R_2=H$ ,  $R_3=CH_3$  in positions of 2' and 4')

7.72 g. of 3-diethylamino-7-aminofluoran, 12.36 g. of 2,4-dimethylbenzyl chloride, 8.28 g. of anhydrous potassium carbonate and 80 ml. of toluene are subjected to reaction in a manner similar to that of Example 1.

White crystals

Yield: 9.5 g. (76.5% of theoretical value)

Melting point: 225-228° C.

Results of analysis:  $C_{42}H_{42}N_2O_3$

Calculated: C, 81.03%; H, 6.75%; N, 4.56%

Found: C, 80.51%; H, 6.80%; N, 4.32%.

#### EXAMPLE 7

Preparation of 3-diethylamino-7-bis(2',5'-dimethylbenzyl)aminofluoran (in I,  $R_1=R_2=H$ ,  $R_3=CH_3$  in each position of 2' and 5')

7.72 g. of 3-diethylamino-7-aminofluoran, 12.36 g. of 2,5-dimethylbenzyl chloride, 8.28 g. of anhydrous potassium carbonate, and 80 ml. of toluene are subjected to reaction in a manner similar to that of Example 1.

White crystals

Yield: 10.5 g. (84% of theoretical value)

Melting point: 214-216° C.

Results of analysis:  $C_{42}H_{42}N_2O_3$

Calculated: C, 81.03%; H, 6.75%; N, 4.50%

Found: C, 80.66%; H, 6.75%; N, 4.36%.

#### EXAMPLE 8

Preparation of 3-diethylamino-7-bis(mixed dimethylbenzyl)aminofluoran [in I,  $R_1=R_2=H$ ,  $R_3=CH_3$  (placed in two of any of the positions 2', 3', 4', 5' and 6')] 75

7.72 g. of 3-diethylamino-7-aminofluoran, 12.36 g. of mixed-dimethylbenzyl chloride (it is prepared by chloromethylating mixed xylene with formalin and hydrochloric acid), 8.28 g. of potassium carbonate anhydride and 80 ml. of toluene are subjected to reaction in a manner similar to that of Example 1.

White crystals

Yield: 8.5 g. (68.5% of theoretical value)

Melting point: 225-228° C.

Results of analysis:  $C_{42}H_{42}N_2O_3$

Calculated: C, 81.03%; H, 6.75%; N, 4.50%

Found: C, 80.01%; H, 6.92%; N, 4.31%.

#### EXAMPLE 9

Preparation of 3-diethylamino-6-chloro-7-dibenzylamino fluoran (in I,  $R_1=H$ ,  $R_2=Cl$ ,  $R_3=H$ )

3.4 g. of 3-diethylamino-6-chloro-7-aminofluoran, 5.1 g. of benzyl chloride, 3.18 g. of anhydrous potassium carbonate and 40 ml. of toluene are subjected to reaction in a manner similar to that of Example 1.

Light orange colored white crystals

Yield: 1 g. (22.5% of theoretical value)

Melting point: 100-105° C.

Results of analysis:  $C_{37}H_{33}N_2O_3Cl$

Calculated: C, 75.94%; H, 5.50%; N, 4.66%

Found: C, 75.88%; H, 6.06%; N, 4.13%.

#### EXAMPLE 10

A pressure sensitive copying paper which uses 3-diethylamino-7-bis(2',5'-dimethylbenzyl)aminofluoran (which was obtained in Example 7), as its color former was prepared as follows:

60 g. of gelatin and 60 g. of gum arabic were dissolved in 50 ml. of water at 40° C. Separately 6 g. of 3-diethylamino-7-bis(2',5'-dimethylbenzyl)aminofluoran was dissolved in 150 g. of diphenyl chloride. Then it was added to the aqueous solution of gelatin and gum arabic, and was completely dispersed and emulsified by means of a homo-mixer. To this dispersion was added water at 50° C. to increase the volume of the dispersion to 2000 ml. Then 90 ml. of 10% acetic acid, and water at 50° C. was added with continuous stirring until the weight of the whole was increased to 4 kg. After an hour's stirring, the dispersion was cooled down to below 10° C. with ice water under stirring, and 10% caustic soda was added to adjust its pH to 9. It was then gradually brought back to room temperature. It was applied to the lower surface of the upper leaf and dried.

Separately a solid acid, such as acid clay and phenolic compounds, was applied to the upper surface of the lower leaf.

When copying was effected with the pressure sensitive copying paper consisting of the upper and lower leaves thus prepared, it immediately developed a green image with an excellent light resistance.

#### EXAMPLE 11

A pressure sensitive copying paper which uses the color former obtained in Example 5 was prepared as follows:

By dissolving 4 g. of 3-diethylamino-7-di(3'-methylbenzyl)aminofluoran in 120 g. of diphenyl chloride and treating the resulting solution in the same manner as described in Example 10, an aqueous solution containing dispersed minute capsules was obtained. It was dried, by spraying, into a dust of minute capsules, which were then mixed and dispersed in a 4% xylene solution of a p-phenylphenol-formaldehyde condensation product. This dispersed solution was applied to a sheet of paper and dried to make a pressure sensitive copying paper. When a regional pressure was exerted on the coated paper, it immediately developed a green image having an excellent light resistance.

## EXAMPLE 12

A pressure sensitive copying paper which uses the color former obtained in Example 6 was prepared as follows:

By dissolving 4 g. of 3 - diethylamino - 7-bis(2',4'-dimethylbenzyl)aminofluoran in 120 g. of diphenyl chloride and treating the resulting solution in the same manner as described in Example 10, an aqueous solution containing dispersed minute capsules was obtained. This was mixed and dispersed with 8 g. of minute dust of p-phenol-phenol-formaldehyde condensation product, and further admixed with 40 g. of pulp. Then, after having been diluted with water so that the final solid contents was reduced to 0.5 percent, it was passed over a net of a Fourdrinier to form a sheet of pressure sensitive copying paper. When a regional pressure was exerted on this sheet, it immediately developed a green image with an excellent light resistance.

In Examples 10, 11 and 12 the solvent of low volatility is diphenyl chloride. Substantially similar results are obtained if, in place of the diphenyl chloride, the solvent of low volatility is a lower alkyl diphenyl such as methyl-, ethyl-, and propyl diphenyl or a higher alkyl benzene, such as dodecyl-, decyl-, and octylbenzene, having a boiling point of above 150° C. If the boiling point of the solvent is at least 150° C. it has sufficient low volatility according to the invention.

The solid acid functions as an electron acceptive adsorbent. In lieu of those used in the previous examples zeolite, bentonite, attapulgite and silton can be used with excellent results.

What is claimed is:

1. A pressure sensitive copying paper system which comprises the incorporation in a paper sheet of capsules containing

(a) a dibenzylaminofluoran compound of the formula:



wherein R<sub>1</sub> and R<sub>2</sub> are individually members selected from the group consisting of hydrogen, halogen, and methyl; R<sub>3</sub> is a member selected from the group consisting of hydrogen, halogen and lower alkyl; R<sub>4</sub> and R<sub>5</sub> are individually members selected from the group consisting of methyl and ethyl; and n is an integer of from 1 to 5;

(b) a solvent of low volatility whereby upon the application of pressure to said paper sheet by a writing means, said capsules in the area of said writing

means are caused to burst, whereby said dibenzylaminofluoran is capable of reacting with an acid to form a color localized in the region of said writing means.

2. The pressure sensitive copying paper system of claim 1 wherein said acid is incorporated into the same sheet as said capsules in a solid form.

3. The pressure sensitive copying paper system of claim 1, wherein said acid is contained in a solid form on the upper layer of a second paper sheet, said second paper sheet being immediately beneath the paper sheet containing said capsules.

4. Pressure sensitive copying paper of claim 1 wherein at least one of the substituents R<sub>1</sub>, R<sub>2</sub> and R<sub>3</sub> is halogen or methyl in the case of R<sub>1</sub> and R<sub>2</sub> or halogen or lower alkyl in the case of R<sub>3</sub>.

5. Pressure sensitive copying paper of claim 1 wherein at least one of the substituents R<sub>1</sub>, R<sub>2</sub>, and R<sub>3</sub> is halogen.

6. Pressure sensitive copying paper of claim 1 wherein R<sub>3</sub> is halogen or lower alkyl.

7. Pressure sensitive copying paper of claim 1 wherein said fluoran is 3-dimethylamino-7-dibenzylamino fluoran.

8. Pressure sensitive copying paper of claim 1 wherein said fluoran is 3-diethylamino - 7-bis(dimethylbenzyl)aminofluoran.

9. Pressure sensitive copying paper of claim 1 wherein said fluoran is 3-diethylamino-6-chloro - 7-dibenzylamino fluoran.

10. Pressure sensitive copying paper of claim 1 wherein the fluoran compound is 3 - diethylamino - 6-methyl-7-dibenzylamino fluoran.

11. Pressure sensitive copying paper of claim 1 wherein the fluoran compound is 3-diethylamino-7-di(p-chlorobenzyl)aminofluoran.

12. Pressure sensitive copying paper of claim 1 wherein the fluoran compound is 3-diethylamino-5-methyl-7-dibenzylamino fluoran.

13. Pressure sensitive copying paper of claim 1 wherein the fluoran compound is 3-diethylamino-7-di(3'-methylbenzyl)aminofluoran.

14. Pressure sensitive copying paper of claim 1 wherein the fluoran compound is 3-diethylamino-7-bis(2',3'-dimethylbenzyl)aminofluoran.

15. Pressure sensitive copying paper of claim 1 wherein the fluoran compound is 3-diethylamino-7-bis(2',5'-dimethylbenzyl)aminofluoran.

## References Cited

## UNITED STATES PATENTS

3,501,331 3/1970 Kimura et al. 260—335, X  
3,641,011 2/1972 Lin et al. 117—36.2 X  
3,715,226 2/1973 Lin 117—36.2

THOMAS J. HERBERT, JR., Primary Examiner

U.S. CL. X.R.

117—36.8; 260—335